

May 9, 1950

R. R. LLOYD

2,507,476

ELECTRODEPOSITION OF CHROMIUM

Filed Feb. 4, 1946



## UNITED STATES PATENT OFFICE

2,507,476

## ELECTRODEPOSITION OF CHROMIUM

Rex R. Lloyd, Boulder City, Nev., assignor, by  
mesne assignments, to Crimora Research & De-  
velopment Corporation, New York, N. Y., a cor-  
poration of Virginia

Application February 4, 1946, Serial No. 645,474

2 Claims. (Cl. 204—105)

1

The present invention relates to the preparation of chromium sulfate solution and, more particularly, to the formation from chromite ore of a chromium sulfate solution in a sufficiently pure state so as to render the same suitable for the preparation of chromium plating electrolytes. This application is a continuation in part of application Ser. No. 578,550, filed February 17, 1945, now abandoned.

Heretofore, it has been the practice to dissolve chromite in sulfuric acid and chromic acid, thereby oxidizing the iron of the chromite. Such a solution, however, is unfit for use in chromium plating electrolytes, for example, until the iron and other impurities are removed. Prior methods of removing iron and other impurities from the solution generally have been unsatisfactory.

It is an object of the present invention to provide a satisfactory method of removing iron and other impurities such as aluminum and magnesium from the chromium sulfate solution.

Another aim of the invention is to obtain a solution containing chromium sulfate stabilized in the green modification form.

A further aim of the invention is to provide a method of preparing chromium sulfate solutions from chromite which is suitable for use with an electroplating step whereby the electroplating may be carried out continuously, if desired.

Another aim of the invention is to provide a method of preparing chromium sulfate solution from chromite for use with an electroplating operation whereby the products of electrolysis, i. e., spent electrolyte, may be re-used to form the chromium sulfate solution.

Other advantages and aims of the invention will be apparent from the following description and appended claims.

The figure is a flow sheet illustrating the practice of the method.

In accordance with the present invention, the chromite ore preferably is first ground to a fine state, for example, by wet grinding to less than 200 mesh size, filtering and drying, to facilitate treatment. The finely ground chromite, so prepared, is then digested with sulfuric and chromic acids. This step is indicated in box 1 of the flow sheet. For preferred results, the amount of sulfuric acid used is sufficient to convert all of the metal in the ore to sulfates, while the amount of chromic acid used is slightly in excess of that required to oxidize the iron. In general, a concentrated sulfuric acid of the order of about 65%  $H_2SO_4$ , is required for efficient digestion. Heating

to an elevated temperature to about 120° C. also facilitates digestion.

After digestion has been carried out to a desired degree, preferably to a point where substantially all of the metal is dissolved, the solution of metal sulfates is separated from the undissolved residue in any convenient manner, such as by filtering. This step is indicated in box 2 of the flow sheet. Any undissolved chromite will be retained on the filter along with the residue. Such undissolved chromite may be separated from the residue by known ore dressing means and returned to the digestion step, as indicated by the lines on the flow sheet.

As will be explained more fully hereinafter, it is an advantage of the present invention that the chromic acid and a large part of the sulfuric acid used in the digesting step can be recovered and re-used, when the resulting material is used as an electrolyte for electrowinning chromium. This is indicated by the line running from the cell 10 to the digester 1. Some sodium and ammonium sulphates may be added to the digester solution.

The filtrate obtained after the leaching operation is then preferably combined with additional ammonium and sodium sulphates and heated to a temperature above 70° C. to stabilize the chromic salts in the green modification, a form well-known in the art. This step is indicated by box 3 in the flow sheet.

Following the stabilization of the chromic salts in the green modification, as described above, it is an advantage of the present invention that the undesired constituents of the solution may be readily separated from chromic sulfate in the stabilized green modification. In accordance with the invention, this is accomplished by cooling the solution to a low temperature, such as —5° C. to —10° C. Under such temperature conditions, the iron, aluminum and magnesium present will separate as crystals of complex salts and may be removed, for example, by centrifuging or filtering. These steps are indicated by boxes 4 and 5, respectively, in the flow sheet.

If desired, the resultant partially purified solution containing chromium sulfate may be further improved for use in a chromium electrowinning process by converting the chromic sulfate present into its violet modification. The separation of the chromic sulfate may be effected by crystallization of the violet chromic sulfate and may be accomplished by crystallization induced by the well-known method of seeding with added 55 purified crystals and allowing the solution to

stand for several hours. The term "chromic sulfate" is meant to include any of the various forms of chromic sulfate itself, as well as complexes containing alkali metal sulfates and/or ammonium sulfates. It has been found that the presence of small quantities of potassium and/or ammonium will especially improve the crystallization of the violet chromic sulfate by forming therewith readily crystallizable alums. This step is indicated by box 7 in the flow sheet.

The resulting purified crystals containing chromium sulfate may be separated in a centrifuge indicated by box 8 in the flow sheet. They are now in a form for use in a chromium electro-winning process, such as is described in my co-pending application, Ser. No. 645,473, filed February 4, 1946, wherein sulphates of chromium, ammonium and sodium are employed. As stated in said application, these components are present in the electrolyte in the following proportions:

Sodium 20-40 grams per liter  
Ammonium 30-50 grams per liter  
Chromium 18-60 grams per liter

The sulfate ion is present in an amount at least stoichiometrically equivalent to the sodium, ammonium and chromium. The amounts of the components added to form the feed solution are governed accordingly to replenish the electrolyte. To increase their purity, they may be re-crystallized one or more times. This step is indicated in box 9 of the flow sheet.

The conversion to the violet modification may be catalyzed by the addition of chromous sulfate. Such chromous sulfate may be obtained by utilizing nearly all of the spent catholyte from the electrowinning cell. It is added in sufficient amount to expedite the crystallization of the violet  $\text{Cr}^{+++}$  salts and to improve their purity, and the quantity is not critical. This step is indicated by the line running from the cell box 10 to box 9 marked "spent catholyte." A part of the spent catholyte is not necessary for this purpose and is mixed with the anolyte in the cell, where it serves to reduce part of the chromic acid formed.

The pure crystals are especially suitable for replacing the chromium in the electrolyte, which has been plated out in the electrowinning operation. This replenishment is accomplished by mixing the crystals with a small amount of make-up sodium sulphate and heating to above 70° C. to stabilize the  $\text{Cr}^{+++}$  salts in the green modification. This step is indicated by the line running from box 9 to the stabilizer, box 11 and thence to the cathode compartment of the cell 10.

The method of the present invention may be used to permit continuous or cyclic operation by direct replacement of plated out chromium from readily available chromite ore. The products of electrolysis, other than metal; namely, chromous sulfate, chromic and sulfuric acids may be recycled in accordance with the invention, as described above and shown on the flow sheet, for economy and convenience of operation.

The practice of the invention is capable of many variations by one skilled in the art without departing from the teachings herein, and all such

variations are intended to be included within the scope of the following claims.

What is claimed is:

1. In a process for the preparation of electrolytic chromium utilizing a compartment cell and an electrolyte prepared by treating chromite with sulphuric acid and chromic acid, the steps of utilizing sulphuric acid and chromic acid derived from the anolyte of the compartment cell to provide at least part of the necessary sulphuric and chromic acids, digesting the acids and chromite at approximately 120° C., separating the chromic sulfate and other metallic sulfates dissolved from the chromite from the insoluble residue, adding ammonium sulfate in an amount sufficient to form ammonium sulfate complexes of the chromium and other metallic sulfates present, heating the solution to a temperature above 70° C. and below the temperature at which decomposition occurs, whereby to stabilize the chromium salts in the green modification, cooling the solution to a temperature between -5° and -10° C. to crystallize iron, aluminum and magnesium-ammonium sulfate complexes and separating them from the solution of green chromium sulfate, seeding the solution to obtain the chromium salts in the violet modification, adding a substantial fraction of the spent catholyte to the solution to catalyze the crystallization of violet chromium alum from the solution, re-dissolving the crystallized chromium alum to form an aqueous solution, mixing the chromium alum with sodium sulfate in an amount slightly less than the ammonium content of the alum to form a catholyte solution having 20-40 grams per liter of sodium, 30-50 grams per liter of ammonium, and 18-60 grams per liter of chromium, all in the form of sulfates, heating the catholyte solution to above 70° C. and below the temperature at which decomposition occurs to stabilize the green modification, electrolyzing such solution in the catholyte compartment of an electrolytic cell and forming in the anolyte compartment of such cell chromic and sulphuric acids.
2. In the process as set forth in claim 1, the additional step of centrifuging the catalyzed solution to separate the violet chromium alum therefrom.

REX R. LLOYD.

#### REFERENCES CITED

The following references are of record in the file of this patent:

#### UNITED STATES PATENTS

| Number    | Name        | Date          |
|-----------|-------------|---------------|
| 1,403,960 | Hultman     | Jan. 17, 1922 |
| 1,502,035 | Hasenclaver | July 22, 1924 |

#### FOREIGN PATENTS

| Number  | Country       | Date          |
|---------|---------------|---------------|
| 5,902   | Great Britain | July 9, 1903  |
| 187,636 | Great Britain | Nov. 2, 1922  |
| 198,645 | Great Britain | Dec. 13, 1923 |

#### OTHER REFERENCES

Mellor, Comprehensive Treatise on Inorganic and Theoretical Chemistry, vol. XI (1931), pp. 435, 437, 438.